

March 9, 1937.

R. YAJIMA

2,073,237

INSIDE FROSTED INCANDESCENT ELECTRIC LAMP BULB

Filed Oct. 22, 1934



Rinjiro Yajima  
INVENTOR

BY *Ole Hennicke*  
his ATTORNEY.

## UNITED STATES PATENT OFFICE

2,073,237

INSIDE-FROSTED INCANDESCENT  
ELECTRIC LAMP BULBRinjiro Yajima, Shinagawa-ku, Tokyo, Japan,  
assignor to Todendenkyu Kabushiki Kaisha,  
Tokyo, JapanApplication October 22, 1934, Serial No. 749,481  
In Japan October 31, 1933

2 Claims. (Cl. 41—43)

This invention relates to an inside-frosted incandescent lamp bulb figured by different intensities of frosting and has for its object to produce a bulb having a delightful appearance and being 5 free of any tendency to produce a dazzling effect when lighted.

The half-frosted bulb hitherto used has the frosted and transparent areas separated by the boundary line between them while the frosted 10 bulb having transparent spots has also been used, but in each case the rays pass freely through the transparent portions or spots producing a dazzling brilliancy which is very unpleasant.

This invention has for its object to avoid such 15 disadvantages and to provide a bulb which is frosted throughout its entire inner surface by means of a weak frosting liquid so as not to weaken the bulb, and which is then subjected to an acid-proof material applied to the frosted surface of the bulb to form any desired figure or spot, after which the bulb is once more subjected to a 20 second frosting treatment and finally washed with water or other suitable means to remove the acid-proof material.

If so desired, the process may be modified in 25 such a manner that the bulb is at first figured by an acid-proof material and then subjected to the first frosting treatment, thereafter washing out the said acid-proof material, and finally frosting the entire surface.

The arrangement of the varied areas consisting 30 of different intensity of the frosting produces an effect which is devoid of any dazzle. The dimensions of the areas may be adjusted by density of the frost liquid and the frosting time. As 35 a subsequent frosting reinforces the weakened portions resulting from the first frosting, no further reinforcing treatment such as heating or chemical treatment is required.

If it is desired to have the figure areas appear 40 in a crystalline form, it is contemplated to separate out the peculiar crystal of such a material on the inner surface of the bulb as is stable to the action of the frosting liquid.

For this purpose, the said material, for instance, 5 may be a supersaturated solution of sodium phthalate, which is first applied on the inner surface of the bulb. Then upon cooling the bulb for a short time, the distinct crystals of sodium phthalate are separated out. After the bulb thus treated has been frosted, said crystals are washed out with water, whereby the figures in the peculiar crystalline form will appear. If the brilliancy of the bulb obtained is too strong, the bulb may 10 be frosted once more after the washing out of the crystals. These crystalline figures can also be formed by means of sublimation of naphthalene or phthalic acid.

Thus the incandescent lamp bulb according to 15 the present invention produces an excellent diffusion of beautiful light and entirely prevents any dazzling effect from the bulb because of the difference in brilliancy produced by different intensity of the frosting in the spaced areas.

The drawing shows a front elevational view 20 with a portion broken away of an incandescent lamp according to the invention in which 1 denotes the part twice frosted and 2 the part frosted but once.

Having now fully explained the nature of invention, what I claim is:

1. The herein described process of frosting the 25 inside surface of an incandescent lamp bulb to produce a crystalline form, which process consists in applying a supersaturated solution of sodium phthalate to the inner surface of the glass bulb, thereafter cooling the same to separate the crystals of sodium phthalate, then frosting the surface between the crystals and finally washing away the crystals to leave the surfaces in the clear 30 where the crystals had been located before being washed away.

2. A process of frosting lamp bulbs, as claimed 35 in claim 1, including this added step of refrosting the inner surface to increase the density of the first frosting and to frost the clear surfaces covered by the crystals during the first frosting.

RINJIRO YAJIMA.